

H. M. SHIMER.  
METHOD AND MEANS FOR REFINING METALS.  
APPLICATION FILED JAN. 26, 1920.

1,403,349.

Patented Jan. 10, 1922.



# UNITED STATES PATENT OFFICE.

HERBERT M. SHIMER, OF PHILADELPHIA, PENNSYLVANIA.

## METHOD AND MEANS FOR REFINING METALS.

1,403,349.

Specification of Letters Patent. Patented Jan. 10, 1922.

Application filed January 26, 1920. Serial No. 354,191.

To all whom it may concern:

Be it known that I, HERBERT M. SHIMER, a citizen of the United States, and resident of Philadelphia, county of Philadelphia, and 5 State of Pennsylvania, have invented an Improvement in Methods and Means for Refining Metals, of which the following is a specification.

The object of my invention is to provide 10 a method and means for refining metals of relatively low fusibility and high volatility, whereby there shall be a substantially perfect refinement and minimum loss.

Heretofore the refining of aluminum, zinc 15 and similar metals and alloys thereof and especially in reclaiming aluminum from barrings and other waste arising from machine work upon castings or other worn out castings, etc., has been attended with imperfect results and very considerable loss owing to 20 the freedom with which they oxidize and volatilize, and it is an object of my invention to eliminate these objectionable results and thereby not only insure great saving 25 by increasing the quantity of the recoveries, but also obtaining a cleaner and purer product as a result of my improved process.

In carrying out my improved process, I 30 fuse and melt within a crucible or furnace pot from which air is excluded, the metal or alloy to be treated; and during said melting subsequent treatment, prior to casting or drawing off the product, subjecting the molten metal or alloy being treated to a 35 suitable flux in an atmosphere which will prevent material oxidation and preferably insure a "reducing" influence upon the molten metal during and preferably throughout the melting and refining operations.

40 My improved method and apparatus are more fully described hereinafter and defined in the claims, the description being had in connection with the accompanying drawings, in which:

45 Fig. 1 is a vertical section of a refining furnace embodying my improvements and in which to practice my improved process; and Fig. 2 is a transverse sectional view of the same, taken in a vertical plane in the direction of line  $z-z$  of Fig. 1.

50 2 is the furnace proper, preferably made of firebrick and provided near the lower part with a suitable oil or gas burner 9 or other source of heat. The burner shown, 55 comprises a mixer and jet producing body 9

having a controlled supply pipe 10 for oil or gas and a controlled blast pipe for compressed air or steam. 12 is a control valve for regulation of the burner as to the extent of the flame produced. 60

3 is a large crucible arranged within the furnace chamber and supported in an oblique position, such that its lower or bottom end is sustained upon the base or pedestal 4 of firebrick and its neck or throat 5 is 65 extended through the front wall 14 at 15. The lower and large body portion of the crucible extends through the opening 13 in the rear wall of the furnace, and near its lowest part it is provided with a casting 70 aperture 7, which may be sealed with fire clay 8 during the melting and refining operation and the seal broken when casting the content of the crucible.

The crucible 3 is filled or charged through 75 the neck 5; and before the melting operation begins, the neck is filled with a stopper or fire clay plug and may be fitted with fire clay sufficiently to prevent entrance of air into the crucible, or too free escape of the 80 gases from within the crucible chamber 20.

17 are tuyeres fitted into apertures 19 formed in the upper part of the crucible above the level of the liquid content thereof; and these tuyeres are connected with any 85 form a continuation of a superheating coil or manifold 16, through which steam or other gaseous medium is supplied to the tuyeres and under the control of a valve 18.

I have found steam, when superheated in 90 the coil 16, to be suitable for the atmosphere within the crucible or pot containing the molten metal and as a means to prevent inflow of air. In practice the air within the crucible may be displaced with the steam as 95 the preliminary operation and before or after the charge is introduced and the neck of the crucible is sealed. It is not essential that the crucible be hermetically sealed as a reasonably tight sealing will insure satisfactory and efficient results, though the best results may be obtained when the sealing is well made during the period in which the metal is in the molten condition. 100

The temperature to be provided by the 105 burner 9 or other source of heat may be varied according to the metal or alloy to be melted and refined and I do not restrict myself in this respect.

By superheating the steam in coil 16, it 110

is brought to a condition of dissociation when admitted to the crucible and, aside from its utilization in blowing out the air from the crucible, the oxygen of the steam which remains is readily taken up by the carbon which may be present in the crucible, whether from the graphite of the crucible itself, from carbon in the charge, or dissociated carbon from the oil mixed with the metal turnings or scrap constituting the metal element of the charge. The oxygen is thus converted into carbonic acid and remains as an inert part of the gaseous content of the crucible, or it may be absorbed in or combined with the fluxes introduced or slag produced according to specific employment of my invention. In any event, whether the carbonic acid remains as an inert gas or in any other combination, the reducing and quantity of it is not a material matter affecting the refining operation.

The hydrogen dissociated from the oxygen of the steam provides a reducing atmosphere and protects the metal from combination with other elements which may be present. The oil present in the metal turnings or scrap being melted will provide hydro-carbons which may provide additional hydrogen in the event of its carbon becoming combined with the oxygen, as before pointed out. The result, in any event, is to provide a reducing atmosphere within the crucible which is maintained throughout the refining process.

35 By sealing the crucible or melting pot during the melting and refining process, the volatile vapors arising from the metals being treated are prevented from escaping and as the gases also are prevented from escaping 40 to an extent which would freely admit the atmospheric air no losses in metal from this cause are permitted and hence the entire metal content of the charge remains and insures a maximum metal output possible.

45 By supplying superheated steam under pressure to the sealed crucible or melting pot, this pressure is exerted upon the molten mass and raises the volatilizing temperature and thereby permits the refining to be carried 50 on efficiently at a higher temperature than that at which the metal normally volatilizes under atmospheric pressure. The result of this treatment at higher temperature is to secure better refining action and a purer 55 product. The melting and refining under a confined gaseous atmosphere incapable of injurious effect upon the metal content, enables the process to be carried on for any period desired without loss from escaping 60 metallic vapors, or their conversion into compounds which enter the slag, and this feature of the invention is especially important. That the refining takes place in a "reducing" atmosphere is also of much importance,

since it tends to eliminate the tendency of 65 metal compounds to be formed with associated matters of the charge and especially from first forming oxides and other metal consuming compounds, as is always liable in open crucible refining.

70 My invention has particular utility in refining aluminum scrap, which may be largely the resulting waste from turning, boring and planing aluminum castings, and as these usually contain oil from the machine shop, 75 they provide part of the carbon and hydro-carbon elements which are advantageous to my process, as before pointed out. If desired, a further quantity of carbon may be 80 employed as a part of the charge and incorporated with the flux, which may be of any usual character and suitable for collecting the foreign substances to be removed from the metal being refined. I have found that 85 during refining the addition of one-half to one per cent of crystal chloride and zinc as a flux to the charge will quickly cause the pasty aluminum mass to become fluid with the liberation of chlorin and under the refining process make the fluid aluminum separate to a position beneath the slag.

90 After the metal charge has been subjected to the preliminary refining temperature within the confines of the crucible or vessel with the air blown out and while under the influence of the reducing atmosphere (preferably of a pressure above atmospheric pressure), whereby the metal is melted and reduced to a clean and pure condition. The 95 casting aperture 7 may be then opened by removing the sealing plug 8 and the pure metal completely cast, without disturbance and inferior results such as would result if the crucible were tilted to pour the metal from beneath the slag. After the metal has been 100 fully run off, the slag may be cast through the same orifice; and where there is not an excess of slag, the same may remain in the crucible with the next "heat" without detriment.

105 While I have found that superheated steam is suitable for the atmosphere within the crucible or melting vessel during refining, I do not confine myself thereto, as any inert gaseous medium may be employed, such 110 as hydrogen, nitrogen, carbonic acid and carbonic oxide, as examples. It will further be understood that a suitable gas may be provided within the vessel by supplying a medium as carbon, oil, grease or flux to the charge before sealing and, after gasifying, 115 maintaining the pressure by steam or other gas supplied by the tuyeres, either superheated or otherwise, as desired.

120 While my process is particularly useful in recovering and refining aluminum, it may be employed in the refining of zinc and all 125 metals having a low volatilizing temperature

or where volatile metallic compounds are formed and which would escape with loss except for the non-oxidizing atmosphere of the crucible or sealed compartment in which 5 they are subjected to treatment.

I have described my improved method and means in that particularity which I deem to be the best exposition of my invention, and that which I prefer in commercial practice, but I do not restrict or confine myself to the minor or secondary details, as such variations may be resorted to as matters of mechanical skill and without a departure from the spirit of the invention.

Having thus described my invention, what I claim as new and desire to secure by Letters Patent, is:—

1. The herein described process for recovery and refining of metals having low 20 volatility, which consists in confining the metallic charge including a reducing material within a melting vessel from which the atmosphere is substantially excluded, subjecting the vessel and its charge to a temperature sufficient to fuse the metallic charge 25 to a pasty condition and while doing so introducing a gaseous atmosphere to prevent inflow of air, introducing a suitable flux capable of bringing the pasty mass to a fluid 30 state at a higher temperature and during this action continuing the maintenance of the gaseous atmosphere to prevent inflow of air, and finally casting the metal separate from the slag.

2. The invention according to claim 1, wherein the charge includes carbon and the air is excluded from the vessel by an atmosphere therein composed of gases of carbonaceous character, hydrogen and hydrocarbons resulting from the action of superheated steam upon the carbon of the charge.

3. The invention according to claim 1, further characterized by providing the metallic charge with carbon and supplying 45 superheated steam to the vessel to blow out the air and in effect seal it against the entrance of air, and after heating the vessel to bring the metal to a pasty condition under a continued pressure in excess of 50 atmospheric pressure during the refining operation, adding a chloride flux to bring the mass to a fluid condition.

4. The invention according to claim 1, further characterized by providing aluminum scrap and carbon as the metallic charge, and crystal chloride of zinc as the flux to raise its temperature and render the charge fluid, vigorously stirring the fluid content of the vessel during the refining 60 operation and at the same time maintaining

the gases within the vessel at a pressure above atmospheric pressure.

5. The process for refining metals, which consists in heating a metal to a temperature higher than its volatilizing temperature 65 while confined within a closed vessel, maintaining a heated gaseous medium within the closed vessel above the molten metal to exclude atmospheric air during the fusing and refining operation, drawing off the refined molten metal from the lower part of the vessel, and maintaining the atmosphere within the vessel at a pressure above atmospheric pressure during the drawing off or casting of the metal from the vessel to maintain the temperature and facilitate the casting 70 flow of the metal.

6. The process of refining metals, which consists in melting a metal of low volatility within a sealed vessel and maintaining within 80 the vessel a gaseous atmosphere above the molten metal having constituents which do not materially combine with the metal, maintaining the molten metal in the sealed vessel under continued pressure and at a 85 temperature above its volatilizing temperature until it reaches a condition of refined purity, and thereafter casting the metal.

7. In a refining furnace, a stationary vessel having a body portion for containing the 90 metallic charge to be refined, said vessel provided with a casting orifice at its upper part inclined to one side of the body portion, a furnace containing the body portion of the vessel and exposing both the charging orifice 95 and the casting orifice, and means for maintaining a supply of a suitable gaseous medium to the upper part of the body portion of the vessel so as to be above the molten metal therein and also to one side of the charging 100 orifice.

8. The invention according to claim 7, further characterized by the vessel being formed of crucible shape, set obliquely across the furnace with its neck extending through the furnace wall and having a removable sealing plug, and the means for supplying the gas to the interior of the vessel comprising a tuyeres fixedly opening 105 through the upper wall of the vessel and leading to a source of superheated gaseous medium outside of the furnace.

9. The invention according to claim 8, wherein the super-heating means comprise suitable coils within the furnace and having 110 a tuyere connection opening through the upper wall structure of the vessel.

In testimony of which invention, I hereunto set my hand.

HERBERT M. SHIMER.